

Dec. 8, 1959

S. VERNET ET AL

2,915,899

HIGH TEMPERATURE MATERIAL

Filed May 18, 1956



INVENTORS  
SERGIUS VERNET  
JAMES FAY CORWIN  
GEORGE ASAKAWA  
BY *SMITH, OLSEN, LEWIS & MCRAE*  
ATTORNEYS

## HIGH TEMPERATURE MATERIAL

Sergius Vernet, James Fay Corwin, and George Asakawa, Yellow Springs, Ohio, assignors, by direct and mesne assignments, to Antioch College, Yellow Springs, Ohio, a corporation of Ohio

Application May 18, 1956, Serial No. 585,891

6 Claims. (Cl. 73—368.2)

This invention relates to thermally expansible materials, and to power elements of the type disclosed in co-pending patent applications, Serial No. 551,829, filed on December 8, 1955 and Serial No. 510,708, filed on May 24, 1955. Such power elements are commonly employed to operate switches and valves.

Objects of the invention are to provide thermal expansion materials having relatively large total expansion and good resistance to chemical decomposition at their expansion temperatures.

Other objects of this invention will appear in the following description and appended claims, reference being had to the accompanying drawings forming a part of this specification wherein like reference characters designate corresponding parts in the several views.

In the drawings:

The single figure is a sectional view through a power element incorporating the invention.

Before explaining the present invention in detail, it is to be understood that the invention is not limited in its application to the details of construction and arrangement of parts illustrated in the accompanying drawings, since the invention is capable of other embodiments and of being practiced or carried out in various ways. Also, it is to be understood that the phraseology or terminology employed herein is for the purpose of description and not of limitation.

In the drawings there is shown a power element 1 including a casing 2, a body or pellet of thermally expansible material 3, a movable wall or piston 4, a corrugated stainless steel diaphragm 5, and a body of pliable force-transmitting material 6. Material 6 is preferably the pliable material disclosed in Serial No. 583,881, filed May 9, 1956, and now abandoned. A disc 7 of polytetrafluoroethylene is positioned between material 6 and piston 4 in order to prevent material 6 from extruding into the clearance space 9 between piston 4 and bore 8. A spring (not shown) is provided for returning piston 4 to its illustrated position during contractive movement of material 3.

Operation of the power element is such that during temperature increase in the ambient atmosphere, material 3 expands against diaphragm 5 so as to force material 6 upwardly in bore 8 and thereby propel piston 4 outwardly against the aforementioned spring. During temperature decrease in the atmosphere material 3 contracts so as to allow the spring to return piston 4 downwardly to its illustrated position.

For many applications it is desirable that material 3 have a relatively large total expansion. Such a large total expansion gives piston 4 a relatively long stroke per given size power element, or in the alternative permits a reduction in power element size required to effect a given piston movement.

Expansion material 3 in the illustrated embodiment is particularly chosen to give a relatively large total expansion. Material 3 includes a mixture of thermally

expansible material and discrete particles of heat-conducting copper, preferably in a volume ratio of about 75% expansible material and 25% copper. The copper particles are evenly dispersed throughout the expansible material so as to quickly and evenly conduct heat from the atmosphere through the expansible material and thereby cause piston 4 to be moved quickly in response to temperature change in the atmosphere.

The expansible materials of the present invention are 10 solid aromatic or "ring" compounds of a "symmetrical" character, i.e. any substituted atom or radical at one position on a ring is balanced by one or more similar elements or radicals at opposite points on the ring. It has been found that the "symmetrical" nature of the 15 chosen compounds permits the individual molecules to "pack" or "fit" close together in the solid state. As a result there are more molecules available for expansion during temperature increase, and the material therefore undergoes a relatively large total expansion.

20 The expansible material may be 1, 2, 4, 5 tetrahalogenated benzene or 1, 3, 5 trihalogenated benzene or 4—4 dihalogenated biphenyl or naphthalene or fluorene. The halogen in the three above mentioned halogenated compounds is preferably bromine or chlorine. Mixtures 25 of 1, 2, 4, 5 tetrabromobenzene and 1, 2, 4, 5 tetrachlorobenzene may be used to give expansion temperature ranges intermediate that of pure 1, 2, 4, 5 tetrabromobenzene and pure 1, 2, 4, 5 tetrachlorobenzene. Similarly mixtures of 1, 3, 5 tribromobenzene and 1, 3, 5 30 trichlorobenzene may be employed to give expansion temperature ranges intermediate that of pure tribromobenzene and pure trichlorobenzene. Combinations of dichlorobiphenyl and dibromobiphenyl may also be employed in a similar manner. In each case where a mixture 35 of materials is employed the expansion temperature range will be determined according to the relative amounts of the component materials being employed.

In the foregoing specification the expansion materials have been described with reference to their use in power elements of the type which are responsive to ambient temperature changes. However it is also contemplated that the expansion materials can be employed in power elements of the type which are responsive to changes in electric current, as for example the power elements disclosed in aforementioned patent application, Serial No. 40 551,829. It will be understood therefore that the term "power element" as used herein, refers both to temperature responsive devices and electric current responsive devices.

50 We claim:

1. A thermally expansible pellet formed as a three dimensional body comprised of heat-conducting material dispersed within a solid expansion material transformable to a liquid in its operating range; said expansion material being selected from the group consisting of 55 1, 2, 4, 5 tetrahalogenated benzene; 1, 3, 5 trihalogenated benzene; 4—4 dihalogenated biphenyl; and fluorene.
2. The combination of claim 1 wherein the expansion material is 1, 2, 4, 5 tetrabromobenzene and 1, 2, 4, 5 tetrachlorobenzene.
3. The combination of claim 1 wherein the expansion material is 1, 2, 4, 5 tetrahalogenated benzene.
4. The combination of claim 1 wherein the expansion material is 1, 3, 5 trihalogenated benzene.
5. The combination of claim 1 wherein the expansion material is 4—4 dibromobiphenyl.
6. The combination of claim 1 wherein the expansion material is fluorene.

70

(References on following page)

## References Cited in the file of this patent

## UNITED STATES PATENTS

|           |               |               |           |
|-----------|---------------|---------------|-----------|
| 2,115,501 | Vernet        | Apr. 26, 1938 | 2,271,307 |
| 2,128,274 | Vernet        | Aug. 30, 1938 | 2,303,348 |
| 2,259,846 | Vernet et al. | Oct. 21, 1941 | 2,368,182 |
| 2,265,586 | Vernet        | Dec. 9, 1941  | 2,534,497 |

|                |               |
|----------------|---------------|
| Ray            | Jan. 27, 1942 |
| Freeman et al. | Dec. 1, 1942  |
| Vernet         | Jan. 30, 1945 |
| Albright       | Dec. 19, 1950 |
| Albright       | Feb. 28, 1956 |
| Woods          | June 24, 1958 |